# EUROPEAN PATENT SPECIFICATION

(11) **EP 0 372 622 B1**
(45) Date of publication and mention of the grant of the patent: **12.04.1995**
(21) Application number: 89203017.2
(22) Date of filing: 28.11.1989
(51) Int. Cl.: D01F 6/18, D01D 5/06, D01F 9/22, D01F 6/38

(54) **Acrylic precursor for carbon fibres and method for its preparation**
Acrylvorläufer für Kohlenstoffasern und Verfahren zur Herstellung derselben
Précurseur acrylique pour fibres de carbone et son procédé de fabrication

(30) Priority: 02.12.1988 IT 2283688
(43) Date of publication of application: 13.06.1990
(73) Proprietor: ENICHEM FIBRE S.p.A., 90139 Palermo (IT)
(72) Inventor: Tasselli, Franco, I-75023 Montalbano Ionico, Matera (IT); Cognigni,Franco, I-20097 San Donato Milanese, Milan (IT); Di Bonito, Renato, I-80121 Naples (IT); Mariano, Armando, I-75100 Matera (IT)
(74) Representative: Fusina, Gerolamo

(56) References cited:
- EP-A- 0 044 534
- EP-A- 0 223 199
- EP-A- 0 255 109
- JP-B-52 039 455
- US-A- 4 349 523

## Description

This invention relates to an acrylic precursor for carbon fibres, to carbon fibres obtained from the precursor, and to a wet spinning process for acrylonitrile copolymers in a polar solvent solution, in particular dimethylacetamide, for producing an acrylic yarn of high mechanical characteristics suitable for conversion into carbon fibres (C. F.)

The production of acrylic yarns suitable for conversion into carbon fibres is known and widely described in the patent and scientific literature. Such yarns are generally known as "acrylic precursors for carbon fibres" because of their specific use.

The methods mostly used for producing acrylic precursors are mainly the wet spinning of solutions of suitable acrylic polymers in organic or inorganic solvents. The organic solvents mostly used include polar compounds of high solvent power towards acrylic polymers, such as dimethylformamide, dimethylacetamide, dimethyl sulphoxide, ethylene carbonate etc.

Widely used inorganic solvents include aqueous sodium thiocyanate solutions, aqueous zinc chloride solutions and concentrated aqueous nitric acid solutions.

In all cases of the known art, these solutions are spun by passage through multi-orifice spinnerets with a orifice diameter of between 50 and 200 »m, the filaments then being coagulated by passage through a bath of suitable non-solvent liquid. The acrylic precursor production process is completed by stretching the yarns generally at high temperature (80-120°C) by their passage about rollers rotating at constant speed, after which they are washed, dried and finally collected. Known acrylic precursor production processes which have proved particularly interesting are those described in US patents 3,993,719 and 4,154,807, which use the wet-dry spinning method. This consists of maintaining the spinneret not in immediate contact with the coagulating bath, so that the dope leaving the spinneret has to pass a few millimetres through the air before being immersed in the bath. This process enables a high spinneret stretch to be obtained.

The patent literature also describes methods for increasing the orientation of the yarn and thus the mechanical characteristics of the acrylic precursor obtained.

These methods are based on further considerable stretch applied to the fibre after the consolidation and drying stage, and thus following the coagulation and initial stretching stages.

The polymers most widely used for forming the solutions used in those spinning processes of the known art for the preparation of carbon fibre acrylic precursors are those which contain one or more monomer units of the following list: methyl acrylate, methyl methacrylate, acrylic acid, methacrylic acid, itaconic acid etc., copolymerized with the acrylonitrile.

With the spinning processes of the known art and using acrylic copolymer solutions of the aforesaid type, acrylic precursors are generally obtained having a maximum tenacity of 50-55 cN/tex and generally containing defects, this having a certain importance with regard to the characteristics of the carbon fibres deriving from them.

The defects depend on the type of spinning process used.

In spinning processes in inorganic solvents, metal residues (such as sodium and zinc) always remain on the fibre, and are deleterious when the acrylic fibre is used in the production of carbon fibre, this as stated being the specific product obtainable from this type of fibre. In this respect, the metal residues contained in the acrylic precursor prejudice the proper progress of the acrylic fibre carbonization stage and lessen the oxidation resistance of the carbon fibre obtained thereby.

In addition the solvent recovery process is very complicated and costly. An inorganic solvent also leads to frequent corrosion problems for the spinning plant.

The maximum tenacity attainable in fibres produced by spinning processes in inorganic solvents is 50-55 cN/tex even when air stretching at the exit from the spinneret is used as described in the aforesaid US patents plus extra stretching after the fibre consolidation as stated.

The technique of stretching at the spinneret exit is not easily applicable to the production of tows containing a large number of filaments (obtainable by suitable spinnerets) because of the danger of the individual filaments adhering together, in that on leaving the spinneret orifices they are still in a non-consolidated gelled solution state.

The spinning processes for acrylic polymer solutions in organic solvents generally produce acrylic precursors in which the structural characteristic are generally worse that for the same precursors obtained from solutions in an inorganic solvent because of the presence of possibly large cavities (macrovoids).

Moreover, these latter generally have an irregular cross-section in the shape of a bean or kidney instead of a circular cross-section which would provide better mechanical properties for the fibre, and would therefore allow more uniform progress of the oxidation process which precedes the carbonization stage in the production of carbon fibres.

The drawbacks of the said known art are well obviated by the spinning method for acrylic polymer solutions according to the present invention, which enables an acrylic precursor yarn to be obtained with very good mechanical characteristics, a perfectly circular filament cross-section free of voids, and a metal impurity content of less than 220 ppm (parts per million).

The acrylic precursor of the present invention is further characterised by a compact fibre structure free of flaws, a regular filament count, a constant count of the various filaments and good separation between them.

The present invention also relates to the acrylic fibres produced by the method and the carbon fibres deriving from them by oxidation and subsequent carbonization, in accordance with the well known processes of the state of the art.

The spinning process is of the wet type comprising the use of solutions of an acrylic polymer of the type described hereinafter in a suitable polar solvent.

According to this process, the acrylic polymer solutions are carefully purified of any impurities which may be present by filtration through two or three napped cotton cloths or metal meshes having mesh apertures of 5-10 »m, and are then fed to the spinning section.

Spinning is carried out by spinnerets containing between 3000 and 40000 orifices, with a capillary diameter variable between 120 and 180 »m and immersed in the coagulating bath.

The process is characterised essentially by the coagulation stage, which is conducted under such bath temperature, time and composition conditions as to obtain at the end of the process an acrylic yarn having the aforesaid characteristics and tenacity values which have never been encountered in acrylic fibres forming part of the known art.

In accordance with the aforesaid, the yarns leaving the spinneret are passed into a coagulating bath maintained at a temperature of between 15 and 35°C and consisting of a binary solvent-non solvent mixture in which the solvent is that of the acrylic polymer solution and the non-solvent is water.

The binary solvent-non solvent mixture has a rigorously controlled composition with a solvent content of between 78 and 82% by weight, and preferably a solvent content which is a fixed value within this range and strays from this value by not more than ± 0.5%. The stretch in the spinneret during coagulation is 1.5-5 times the solution extrusion rate through the spinneret orifices.

After coagulation, the yarn passes about a roller rotating at a peripheral speed of 4-10 m/minute and is stretched in air at ambient temperature to the extent of between 2 and 3 times by passage about a second roller rotating at a peripheral speed of between 2 and 3 times that of the preceding roller.

The yarn is then washed in countercurrent with demineralized water at a temperature of between 20°C and 50°C and is again stretched from 3 to 6 times in a water bath maintained at a temperature of between 98 and 105°C.

The subsequent stages in the wet spinning process according to the present invention comprise lubrication, consisting of passing the yarn through a bath containing a lubricant and an antistatic agent, drying by passage over rollers heated to a temperature of between 100 and 150°C and preferably between 130 and 140°C, and further stretching to the extent of 1.2-1.5 times at temperatures between 120 and 170°C and thermal stabilization by contact with hot rollers or heating elements heated to 120-170°C.

The yarn collection rate on the bobbins is between 50 and 80 m/minute.

The aforesaid sequence of operations plus a proper choice of process parameters such as the solution concentrations, the temperatures of the various process stages, the stretch in the spinneret, the coagulation conditions and the total stretch conditions enable acrylic fibres to be obtained having a tenacity of between 60 and 75 cN/tex, these being values with which the corresponding tenacity values obtained by spinning the same polymer solutions in the known processes of the state of the art in no way compare.

Furthermore, the fibres obtained by the spinning process according to the present invention have perfectly round cross-sections and an extremely compact structure free of flaws.

Those acrylic polymers which are most widely used in preparing polymer solutions for feeding to the spinnerets are acrylonitrile copolymers (ACN) with one or more acrylic monomers such as acrylic acid, methacrylic acid, methyl acrylate, methyl methacrylate, acrylates and methacrylates in general, itaconic acid and other ethylenically unsaturated monomers able to copolymerize with acrylonitrile.

The preferred copolymers are those of high acrylonitrile content (acrylonitrile content exceeding 90%).

Other preferred copolymers are those of high ACN content containing some percentage (1-10 % by weight) of monomers containing the carboxyl function, such as acrylic acid, methacrylic acid, itaconic acid etc.

The most suitable polymers include acrylonitrile-acrylic acid copolymers containing 94-98% of acrylonitrile, and acrylonitrile-methylacrylate-acrylic acid terpolymers containing from 94-97% of acrylonitrile, 1-3% of acrylic acid and 1-5% of methylacrylate.

These copolymers are prepared by the usual radical polymerization methods well known to the expert of the art.

The acrylic solutions of the said copolymers are formed by dissolving them in a polar solvent of high solvent power. Those particularly preferred are dimethylformamide, dimethylacetamide and dimethylsulphoxide.

The polymer concentration in the spinning solution is a function of its molecular weight.

Preferred polymers are those having a molecular weight corresponding to an MD of 1500-2000 where ${\text{MD = η}}_{\text{spec}} \text{.1000/C}$ (η_{spec} is the specific viscosity in dimethylformamide measured at 35°C and C the concentration in g/100 c.c.).

As stated heretofore, the specific application of the "acrylic precursors" produced by the method according to the present invention is the production of carbon fibres by carbonization methods well known in the state of the art.

The use of acrylic precursors produced by the method of the present invention enables carbon fibres having excellent mechanical characteristics to be obtained, while using thermal oxidation temperatures for the acrylic fibres (this being a well known stage in the carbonization process) which are relatively low and for shorter times.

For example, an acrylic precursor consisting of an acrylonitrile (ACN) - methylacrylate (MA) - acrylic acid (AA) terpolymer containing 94% of ACN, 2% of AA and 4% of MA, processed in a carbon fibre production plant by way of a first oxidation stage in air at a temperature of 220-240°C and two carbonization stages in an inert environment (nitrogen) with a maximum temperature of 1500°C, resulted in carbon fibres with the following characteristics:

| | |
|---|---|
| Tenacity | ≧ 3.5 GPa |
| Modulus | 220-270 Pa |
| Elongation | 1-1.7% |
| Density | 1.75-1.78 |
| Carbon percentage | 95-96% |

The following examples illustrate the invention but must in no way be considered as limitative of its scope.

### EXAMPLE 1

### a) Polymer preparation

The following reactants were continuously fed to a continuous aqueous suspension polymerization plant comprising three reactors in cascade:
a - acrylonitrile
b - methyl acrylate
c - aqueous solution of acrylic acid
d - aqueous solution of H₂SO₄
e- aqueous solution of sodium hydroxylamine sulphonate
f - aqueous solution of sodium bisulphite.

The feed rates were such as to satisfy the following ratios: Monomer composition: 94.5% ACN, 3.5% MA, 2% AA; Catalysts: 0.6% of sodium hydroxylamine sulphonate and 1.5% of sodium bisulphite on the monomers; Aqueous H₂SO₄ solution such as to maintain the reaction pH at 2.5; Ratio H₂O/monomers: 5.5/1; Total reaction time 9 hours; Reaction temperature 55°C; Conversion 92%; MD 1800.

The polymer, obtained in the form of a slurry, was filtered through a rotary filter, washed with deionized water until the salts (catalyst residues) had completely disappeared, and dried in a fluidized bed drier.

### b) Solution preparation

The polymer was dispersed in DMAc at -7°C; the polymer slurry was then transformed into a solution by heating in a plate heat exchanger at 88°C.

The polymer solution obtained, containing 23% of solids, was carefully filtered in a filter press through suitable filter cloths consisting of cotton linters (1st stage), 20 »m aperture metal cloth (2nd stage), and 10 »m aperture metal cloth (3rd stage).

### c) Spinning

The polymer solution from the filtration stage was then spun in a wet spinning plant under the following spinning conditions:
- Temperature of polymer solution at spinneret inlet 50°C.
- Circular spinneret 80 mm diameter with 6000 orifices of 150 »m in diameter.
- Coagulating bath consisting of an aqueous 80% solution of dimethylacetamide maintained at 24°C.
- Collection rate after coagulation 5 metres/minute.
- Stretch in spinneret 2.4
- Stretch in air through two pairs of rollers, stretching 2.5 times.
- Countercurrent washing in 4 stages with deionized water at 45-50°C.
- Stretch in water at 98°C, stretching 4 times.
- Lubrication with aqueous solution of Span 60 + Tween 60 + G 265 (Trade Marks) of Atlas in ratio 3:1:1.
- Yarn drying under tension over steam heated rollers at maximum temperature of 130°C.
- Further stretching under dry conditions over rollers heated to 140°C with stretching 1.4 times.
- Stabilization over hot rollers at 140°C.
- Yarn collection under constant tension at a rate of about 70 metres/minute.

The characteristics of the obtained fibre were as follows:

| | |
|---|---|
| Total yarn count | 7,200 dtex |
| Filament count | 1.2 dtex |
| Tenacity | 70 cN/tex |
| Elongation | 13% |
| H₂O regain 100°C | 10% |
| Finish percentage | 0.3% |
| Sodium | 100 ppm |
| Filament cross-section | circular |
| Voids after coagulation | 0 |
| Flaws in finished fibre | 0 (see photographs, enclosures 1 and 2: cross-sections through final fibre). |

### EXAMPLE 2 (Comparative)

The polymer solution of Example 1 was spun under the following spinning conditions:
- Spinneret 6000 orifices, orifice diameter 52 »m.
- Coagulating bath: aqueous 50% solution of dimethylacetamide maintained at 45°C.
- Collection rate after coagulation 7 metres/minute.
- Stretch in spinneret 0.67
- Stretch in air, not possible.
- Countercurrent washing as in Example 1.
- Stretch in water at 98°C, 7 times (the maximum possible).
- Lubrication, drying, extra stretching and collection as in Example 1.

The fibre characteristics were as follows:

| | |
|---|---|
| Total yarn count | 7,200 dtex |
| Filament count | 1.2 dtex |
| Tenacity | 55 cN/tex |
| Elongation | 14% |
| H₂O regain 100°C | 11% |
| Finish percentage | 0.3% |
| Sodium | 110 ppm |
| Filament cross-section | kidney shaped |
| Voids after coagulation, number/mm | 10-30 |
| Flaws in finished fibre, number/mm | 5-10 (see photographs, enclosures 3 and 4: cross-sections through final fibre). |

The given examples clearly show that the best fibre characteristics are obtained under the spinning conditions suggested by our invention.

### EXAMPLE 3

The fibres produced in Examples 1 and 2 are both converted into carbon fibres in an industrial plant operating under the following conditions:
Feed 200 bobbins
Oxidation in two furnaces operating in 4 stages, ie 220, 230, 235, 240°C
Stretch under oxidation 5%
1st carbonization stage in N₂ at 900°C
2nd carbonization stage in N₂ at 1400°C
Surface treatment by electrolysis with an ammonium bicarbonate solution.

Lubrication by aqueous epoxy resin dispersion
Drying at 150°C.

The carbon fibre characteristics were as follows:

| | Precursor Ex. 1 | Precursor Ex. 2 |
|---|---|---|
| Count dtex | 3,600 | 3,600 |
| Tenacity | 3.6 GPa | 3.0 GPa |
| Modulus | 230 GPa | 235 GPa |
| Elongation | 1.5% | 1.3% |

Percentages are expressed by weight, even if not explicitly stated, when indicating contents.

## Claims (Claims for the following Contracting State(s): AT, BE, FR, DE, GB, GR, LU, NL, SE, CH, LI)

1. An acrylic precursor for carbon fibres characterised by:
a) a fibre structure of the individual filaments which is compact and completely free of flaws;
b) a perfectly circular filament cross-section;
c) a maximum metal impurity content of 220 parts per million, expressed as metal in the elemental state;
d) a tenacity greater than or equal to 60 cN/tex;
e) an elongation exceeding 10%;
f) a total yarn count of between 3000 and 500,000 dtex;
g) count of each individual filament between 1 and 1.6 dtex.

2. Carbon fibres obtained from the precursors claimed in the preceding claim, characterised by a tenacity greater than or equal to 3.5 GPa and a modulus greater than or equal to 200 GPa.

3. A method for preparing the carbon fibre acrylic precursors claimed in claim 1, comprising the following stages:
a) wet-spinning a solution of an acrylic copolymer in a polar organic solvent through 120-180 »m diameter orifices of a spinneret immersed in a coagulating bath at a temperature of 15-35°C which contains said solvent in binary solvent-non solvent mixture with water, the mixture composition being rigorously controlled and having an organic solvent content of 78-82% by weight, said content being preferably maintained within said range at a value from which it strays by not more than ± 0.5%, with simultaneous stretching in the spinneret of between 1.5 and 5; said stretching in the spinneret being the ratio of the collection speed after coagulation to the speed with which the polymer solution passes through the spinneret orifices.
b) stretching in air at ambient temperature to the extent of between 2 and 3 times;
c) washing the resultant fibre with countercurrent water;
d) stretching from 3 to 6 times in a water bath maintained at a temperature of between 98 and 105°C;
e) lubrication;
f) drying under tension at a temperature of between 100 and 150°C;
g) stretching from 1.2 to 1.5 times at a temperature of between 120 and 150°C;
h) stabilization under tension at a temperature of between 120 and 170°C;
i) final collection.

4. A method as claimed in the claim 3, wherein the polar organic solvent is chosen from dimethylformamide, dimethylacetamide and dimethylsulphoxide.

5. A method as claimed in claims 3 and 4, wherein the polar solvent is dimethylacetamide.

6. A method as claimed in claim 3, wherein the acrylic polymer is a copolymer of acrylonitrile with one or more monomers chosen from the group comprising acrylates, methacrylates, acrylic acid, methacrylic acid and itaconic acid.

7. A method as claimed in claim 3, wherein the acrylic polymer is a terpolymer of acrylonitrile with methyl acrylate and acrylic acid, and contains at least 94% of acrylonitrile.

8. A method as claimed in claim 3, wherein the coagulating bath of point a) consists preferably of a water/dimethylacetamide binary mixture.

9. A method as claimed in claim 8, wherein the dimethylacetamide content of the binary mixture is preferably 80% by weight.

## Claims (Claims for the following Contracting State(s): ES)

1. A method for preparing an acrylic precursor for carbon fibres having:
a) a fibre structure of the individual filaments which is compact and completely free of flaws;
b) a perfectly circular filament cross-section;
c) a maximum metal impurity content of 220 parts per million, expressed as metal in the elemental state;
d) a tenacity greater than or equal to 60 cN/tex;
e) an elongation exceeding 10%;
f) a total yarn count of between 3000 and 500,000 dtex;
g) count of each individual filament between 1 and 1.6 dtex,
said method consisting in the following stages:
a) wet-spinning a solution of an acrylic copolymer in a polar organic solvent through 120-180 »m diameter orifices of a spinneret immersed in a coagulating bath at a temperature of 15-35°C which contains said solvent in binary solvent non-solvent mixture composition being rigorously controlled and having an organic solvent content of 78-82% by weight, said content being preferably maintained within said range at a value from which it strays by not more than ± 0.5%, with simultaneous stretching in the spinneret of between 1.5 and 5; said stretching in the spinneret being the ratio of the collection speed after coagulation to the speed with which the polymer solution passes through the spinneret orifices.
b) stretching in air at ambient temperature to the extent of between 2 and 3 times;
c) washing the resultant fibre with countercurrent water;
d) stretching from 3 to 6 times in a water bath maintained at a temperature of between 98 and 105°C;
e) lubrication;
f) drying under tension at a temperature of between 100 and 150°C;
g) stretching from 1.2 to 1.5 times at a temperature of between 120 and 150°C;
h) stabilization under tension at a temperature of between 120 and 170°C;
i) final collection.

2. A method as claimed in claim 1, characterized in that carbon fibres obtained from the precursors have a tenacity greater than or equal to 3.5 GPa and a modulus greater than or equal to 200 GPa.

3. A method as claimed in the claim 1, wherein the polar organic solvent is chosen from dimethylformamide, dimethylacetamide and dimethylsulphoxide.

4. A method as claimed in claim 1, wherein the polar solvent is dimethylacetamide.

5. A method as claimed in claim 1, wherein the acrylic polymer is a copolymer of acrylonitrile with one or more monomers chosen from the group comprising acrylates, methacrylates, acrylic acid, methacrylic acid and itaconic acid.

6. A method as claimed in claim 1, wherein the acrylic polymer is a terpolymer of acrylonitrile with methyl acrylate and acrylic acid, and contains at least 94% of acrylonitrile.

7. A method as claimed in claim 1, wherein the coagulating bath of point a) consists preferably of a water/dimethylacetamide binary mixture.

8. A method as claimed in claim 7, wherein the dimethylacetamide content of the binary mixture is preferably 80% by weight.

## Patentansprüche (Patentansprüche für folgende(n) Vertragsstaat(en): AT, BE, FR, DE, GB, GR, LU, NL, SE, CH, LI)

1. Acryl-Vorstufe für Kohlenstoffasern, gekennzeichnet durch:
a) eine Faserstruktur der einzelnen Fäden, die kompakt und vollständig frei von Defekten ist;
b) einen vollständig kreisförmigen Fadenquerschnitt;
c) einen maximalen Gehalt an metallischen Verunreinigungen von 220 ppm, ausgedrückt als Metall im Elementarzustand;
d) eine Festigkeit von mindestens 60 cN/Tex;
e) eine 10% überschreitende Dehnung;
f) eine Gesamtgarnnummer zwischen 3000 und 500000 dtex;
g) eine Nummer eines jeden einzelnen Fadens zwischen 1 und 1,6 dtex.

2. Aus den im vorstehenden Anspruch beanspruchten Vorstufen erhaltene Kohlenstoffasern, gekennzeichnet durch eine Festigkeit von mindestens 3,5 GPa und ein Modul von mindestens 200 GPa.

3. Verfahren zur Herstellung der in Anspruch 1 beanspruchten Acryl-Vorstufen für Kohlenstoffasern, das die folgenden Schritte umfaßt:
a) Naßspinnen einer Lösung eines Acrylcopolymers in einem polaren organischen Lösungmittel durch einen Durchmesser von 120 bis 180 »m aufweisende Öffnungen einer Spinndüse, die in ein Koagulierbad mit einer Temperatur von 15-35°C eingetaucht ist, das das Lösungsmittel in einem binären Lösungsmittel- Nicht-Lösungsmittelgemisch mit Wasser enthält, wobei die Zusammensetzung des Gemisches genau kontrolliert wird und einen Gehalt an organischem Lösungsmittel von 78-82 Gew.-% aufweist, wobei der Gehalt innerhalb des Bereichs vorzugsweise bei einem Wert gehalten wird, um den er um nicht mehr als ±0,5% streut, bei gleichzeitigem Strecken in der Spinndüse um einen Wert zwischen 1,5 und 5; wobei das Strecken in der Spinndüse das Verhältnis der Aufnahmegeschwindigkeit nach dem Koagulieren zur Geschwindigkeit ist, mit der die Polymerlösung durch die Spinndüsenöffnungen hindurchtritt;
b) Strecken in Luft bei Umgebungstemperatur um das 2-3 fache;
c) Waschen der entstandenen Faser mit Wasser im Gegenstrom;
d) Strecken um das 3-6 -fache in einem Wasserbad, das auf einer Temperatur zwischen 98 und 105°C gehalten wird;
e) Schmieren;
f) Trocknen unter Spannung bei einer Temperatur zwischen 100 und 150°C;
g) Strecken um das 1,2 bis 1,5-fache bei einer Temperatur zwischen 120 und 150°C;
h) Verfestigen unter Spannung bei einer Temperatur zwischen 120 und 170°C;
i) End-Aufnahme.

4. Verfahren nach Anspruch 3, wobei das polare organische Lösungsmittel ausgewählt wird aus Dimethylformamid, Dimethylacetamid und Dimethylsulfoxid.

5. Verfahren nach den Ansprüchen 3 und 4, wobei das polare Lösungsmittel Dimethylacetamid ist.

6. Verfahren nach Anspruch 3, wobei das Acrylpolymer ein Copolymer von Acrylnitril mit einem oder mehreren Monomeren ist, die aus der Gruppe ausgewählt werden, die Acrylate, Methacrylate, Acrylsäure, Methacrylsäure und Itaconsäure umfaßt.

7. Verfahren nach Anspruch 3, wobei das Acrylpolymer ein Terpolymer von Acrylnitril mit Methylacrylat und Acrylsäure ist und mindestens 94% Acrylnitril enthält.

8. Verfahren nach Anspruch 3, wobei das Koagulierbad von Punkt a) hauptsächlich aus einem binären Wasser/Dimethylacetamidgemisch besteht.

9. Verfahren nach Anspruch 8, wobei der Dimethylacetamidgehalt des binären Gemisches vorzugsweise 80 Gew.-% beträgt.

## Patentansprüche (Patentansprüche für folgende(n) Vertragsstaat(en): ES)

1. Verfahren zur Herstellung einer Acryl-Vorstufe für Kohlenstoffasern mit:
a) einer Faserstruktur der einzelnen Fäden, die kompakt und vollständig frei von Defekten ist;
b) einem vollständig kreisförmigen Fadenquerschnitt;
c) einem maximalen Gehalt an metallischen Verunreinigungen von 220 ppm, ausgedrückt als Metall im Elementarzustand;
d) einer Festigkeit von mindestens 60 cN/Tex;
e) einer 10% überschreitende Dehnung;
f) einer Garnnummer zwischen 3000 und 500000 dtex;
g) einer Nummer eines jeden einzelnen Fadens zwischen 1 und 1,6 dtex,
wobei das Verfahren die folgenden Schritte aufweist:
a) Naßspinnen einer Lösung eines Acrylcopolymers in einem polaren organischen Lösungmittel durch einen Durchmesser von 120 bis 180 »m aufweisende Öffnungen einer Spinndüse, die in ein Koagulierbad mit einer Temperatur von 15-35°C eingetaucht ist, das das Lösungsmittel in einem binären Gemisch mit Wasser enthält, wobei die Zusammensetzung des Gemisches genau kontrolliert wird und einen Gehalt an organischem Lösungsmittel von 78-82 Gew.-% aufweist, wobei der Gehalt innerhalb des Bereichs vorzugsweise bei einem Wert gehalten wird, um den er um nicht mehr als -+0,5% streut, bei gleichzeitigem Strecken in der Spinndüse um einen Wert zwischen 1,5 und 5; wobei das Strecken in der Spinndüse das Verhältnis der Aufnahmegeschwindigkeit nach dem Koagulieren zur Geschwindigkeit ist, mit der die Polymerlösung durch die Spinndüsenöffnungen hindurchtritt;
b) Strecken in Luft bei Umgebungstemperatur um das 2-3 fache;
c) Waschen der entstandenen Faser mit Wasser im Gegenstrom;
d) Strecken um das 3-6 -fache in einem Wasserbad, das auf einer Temperatur zwischen 98 und 105°C gehalten wird;
e) Schmieren;
f) Trocknen unter Spannung bei einer Temperatur zwischen 100 und 150°C;
g) Strecken um das 1,2 bis 1,5-fache bei einer Temperatur zwischen 120 und 150°C;
h) Verfestigen unter Spannung bei einer Temperatur zwischen 120 und 170°C;
i) End-Aufnahme.

2. Verfahren nach Anspruch 1, dadurch gekennzeichnet, daß aus den Vorstufen erhaltene Kohlenstoffasern eine Festigkeit von mindestens 3,5 GPa und ein Modul von mindestens 200 GPa aufweisen.

3. Verfahren nach Anspruch 1, wobei das polare organische Lösungsmittel ausgewählt wird aus Dimethylformamid, Dimethylacetamid und Dimethylsulfoxid.

4. Verfahren nach den Anspruch 1, wobei das polare Lösungsmittel Dimethylacetamid ist.

5. Verfahren nach Anspruch 1, wobei das Acrylpolymer ein Copolymer von Acrylnitril mit einem oder mehreren Monomeren ist, die aus der Gruppe ausgewählt werden, die Acrylate, Methacrylate, Acrylsäure, Methacrylsäure und Itaconsäure umfaßt.

6. Verfahren nach Anspruch 1, wobei das Acrylpolymer ein Terpolymer von Acrylnitril mit Methylacrylat und Acrylsäure ist und mindestens 94% Acrylnitril enthält.

7. Verfahren nach Anspruch 1, wobei das Koagulierbad von Punkt a) hauptsächlich aus einem binären Wasser/Dimethylacetamidgemisch besteht.

8. Verfahren nach Anspruch 7, wobei der Dimethylacetamidgehalt des binären Gemisches vorzugsweise 80 Gew.-% beträgt.

## Revendications (Revendications pour l'(les) Etat(s) contractant(s) suivant(s): AT, BE, FR, DE, GB, GR, LU, NL, SE, CH, LI)

1. Précurseur acrylique pour des libres de carbone caractérisés par
a) une structure fibreuse des filaments individuels qui est compacte et totalement exempte de défauts.
b) une section transversale du filament parfaitement circulaire,
c) une teneur maximale en impuretés métalliques égale à 220 parties par million, exprimée sous forme de métal à l'état d'élément,
d) une ténacité supérieure ou égale à 60 cN/tex,
e) un allongement supérieur à 10 %,
f) un titre global du filé compris entre 3000 et 500 000 dtex,
g) un titre de chaque filament individuel compris entre 1 et 1,6 dtex.

2. Fibres de carbone obtenues à partir du précurseur conforme à la revendication précédente, caractérisées par une ténacité supérieure ou égale à 3.5 GPa et un module supérieur ou égal à 200 GPa.

3. Procédé pour préparer les précurseurs acryliques de libres de carbone conformes à la revendication 1 comprenant les étapes suivantes :
a) filage à l'humide d'une solution d'un copolymère acrylique dans un solvant organique polaire à travers des orifices, ayant un diamètre compris entre 120 et 180 »m, d'une filière immergée dans un bain coagulant à une température de 15 - 35 °C qui contient ledit solvant et de l'eau sous forme d'un mélange binaire solvant-non solvant, la composition du mélange étant rigoureusement contrôlée et ayant une teneur en solvant organique comprise entre 78 et 82 % en poids, ladite teneur étant de préférence maintenue a l'intérieur de cette fourchette à une valeur de laquelle elle ne dévie pas plus de ± 0,5 %, avec un étirage simultané dans la filière avec un taux d'étirage compris entre 1,5 et 5, ledit taux d'étirage dans la filière correspondant au rapport de la vitesse d'enroulement après coagulation à la vitesse avec laquelle la solution de polymère passe par les orifices de la filière.
b) étirage dans l'air à température ambiante avec un taux d'étirage compris entre 2 et 3,
c) lavage de la libre obtenue avec de l'eau en contre-courant,
d) étirage avec un taux d'étirage de 3 à 6 dans un bain d'eau maintenu à une température de 98 °C à 105 °C,
e) lubrification,
f) séchage sous tension à une température comprise entre 100 °C et 150°C,
g) étirage avec un taux d'étirage de 1,2 à 1,5 à une température comprise entre 120 et 150 °C,
h) stabilisation sous tension à une température comprise entre 120 °C et 170 °C,
i) enroulement final.

4. Procédé conforme à la revendication 3 dans lequel le solvant organique polaire est choisi parmi le diméthylformamide, le diméthylacétamide et le diméthylsulfoxyde.

5. Procédé conforme aux revendications 3 et 4 dans lequel le solvant polaire est le diméthylacétamide.

6. Procédé conforme à la revendication 3 dans lequel le polymère acrylique est un copolymère d'acrylonitrile et d'un ou de plusieurs monomères choisis dans le groupe formé par les acrylates, les méthacrylates, l'acide acrylique, l'acide méthacrylique et l'acide itaconique.

7. Procédé conforme à la revendication 3 dans lequel le polymère acrylique est un terpolymère d'acrylonitrile, d'acrylate de méthyle et d'acide acrylique et contient au moins 94 % d'acrylonitrile.

8. Procédé conforme à la revendication 3 dans lequel le bain coagulant au de l'étape a) est constitué de préférence d'un mélange binaire eau/diméthylacétamide.

9. Procédé conforme à la revendication 8 dans lequel la teneur en diméthylacétamide du mélange binaire est de préférence égale à 80 % en poids.

## Revendications (Revendications pour l'(les) Etat(s) contractant(s) suivant(s): ES)

1. Procédé de préparation d'un précurseur acrylique pour des fibres de carbone ayant
a) une structure fibreuse des filaments individuels qui est compacte et totalement exempte de défauts,
b) une section transversale du filament parfaitement circulaire,
c) une teneur maximale en impuretés métalliques égale à 220 parties par million, exprimée sous forme de métal à l'état d'élément,
d) une ténacité supérieure ou égale à 60 cN/tex.
e) un allongement supérieur à 10 %,
f) un titre global du filé compris entre 3000 et 500 000 dtex,
g) un titre de chaque filament individuel compris entre 1 et 1,6 dtex,
ledit procédé consistant à réaliser les étapes suivantes :
a) filage à l'humide d'une solution d'un copolymère acrylique dans un solvant organique polaire à travers des orifices, ayant un diamètre compris entre 120 et 180 »m, d'une filière immergée dans un bain coagulant à une température de 15 - 35 °C qui contient ledit solvant et de l'eau sous forme d'un mélange binaire solvant-non solvant, la composition du mélange étant rigoureusement contrôlée et ayant une teneur en solvant organique comprise entre 78 et 82 % en poids, ladite teneur étant de préférence maintenue à l'intérieur de cette fourchette à une valeur de laquelle elle ne dévie pas plus de ± 0,5 %, avec un étirage simultané dans la filière avec un taux d'étirage compris entre 1,5 et 5, ledit taux d'étirage dans la filière correspondant au rapport de la vitesse d'enroulement après coagulation à la vitesse avec laquelle la solution de polymère passe par les orifices de la filière.
b) étirage dans l'air à température ambiante avec un taux d'étirage compris entre 2 et 3,
c) lavage de la libre obtenue avec de l'eau en contre-courant,
d) étirage avec un taux d'étirage de 3 à 6 dans un bain d'eau maintenu à une température de 98 °C à 105 °C,
e) lubrification,
f) séchage sous tension à une température comprise entre 100 °C et 150 °C,
g) étirage avec un taux d'étirage de 1,2 à 1,5 à une température comprise entre 120 et 150 °C,
h) stabilisation sous tension à une température comprise entre 120 °C et 170 °C,
i) enroulement final.

2. Procédé conforme à la revendication 1, caractérisé en ce que les fibres de carbone obtenues à partir des précurseurs ont une ténacité supérieure ou égale à 3,5 GPa et un module supérieure ou égal à 200 GPa.

3. Procédé conforme à la revendication 1 dans lequel le solvant organique polaire est choisi parmi le diméthylformamide, le diméthylacétamide et le diméthylsulfoxyde.

4. Procédé conforme à la revendication 1 dans lequel le solvant polaire est le diméthylacétamide.

5. Procédé conforme à la revendication 1 dans lequel le polymère acrylique est un copolymère d'acrylonitrile et d'un ou de plusieurs monomères choisis dans le groupe formé par les acrylates, les méthacrylates, l'acide acrylique, l'acide méthacrylique et l'acide itaconique.

6. Procédé conforme à la revendication 1 dans lequel le polymère acrylique est un terpolymère d'acrylonitrile, d'acrylate de méthyle et d'acide acrylique et contient au moins 94 % d'acrylonitrile.

7. Procédé conforme à la revendication 1 dans lequel le bain coagulant au de l'étape a) est constitué de préférence d'un mélange binaire eau/diméthylacétamide.

8. Procédé conforme à la revendication 7 dans lequel la teneur en diméthylacétamide du mélange binaire est de préférence égale à 80 % en poids.
